

Feb. 16, 1926.

1,573,764

C. N. FORREST

## PROCESS OF TREATING GILSONITE

Filed August 19, 1919



**WITNESSES:**

WITNESSES.

John C. Berger.  
Thomas W. Kerr Jr.

**INVENTOR:**

Charles N. Forrest,  
BY *Talley & Paul*  
ATTORNEYS.

## UNITED STATES PATENT OFFICE.

CHARLES N. FORREST, OF RAHWAY, NEW JERSEY, ASSIGNOR TO THE BARBER ASPHALT COMPANY, OF PHILADELPHIA, PENNSYLVANIA, A CORPORATION OF WEST VIRGINIA.

## PROCESS OF TREATING GILSONITE.

Application filed August 19, 1919. Serial No. 318,536.

To all whom it may concern:

Be it known that I, CHARLES N. FORREST, a citizen of the United States, and a resident of Rahway, in the county of Union and State of New Jersey, have invented certain new and useful Improvements in Processes of Treating Gilsonite, whereof the following is a specification.

My invention relates to gilsonite products and their manufacture, and its object is the production from gilsonite of various useful substances in a commercially practicable and economical way. The novelty of my invention resides not only in my processes and methods of manufacture, but extends, also, to some of the substances obtained, which are in themselves new.

My present application, it will be understood, is in part a continuation of my application, Serial No. 195,721, filed October 10, 1917, under the title "Liquid hydrocarbon".

Gilsonite is a natural solid bitumen, of well known physical properties, including a peculiar, characteristic conchoidal fracture, found principally in certain sections of Utah. As compared with other natural bitumens in their native state, it is remarkable for its very high degree of purity. Its specific gravity at 77° F. varies over a range of, approximately, 1.040 to 1.056. It has been used as an ingredient in paints and varnishes; in paving, waterproofing, and roofing compounds; and in rubber manufacturers.

Of the chemical nature or possibilities of gilsonite, practically nothing is known. Scientific investigations heretofore attempted have been perfunctory, abortive, and inconclusive; and exploitation commercially has not even been attempted.

The vague state of the world's information regarding gilsonite prior to my invention is well illustrated in a paper by Day entitled "Investigation of Utah gilsonite, a variety of asphalt" read June 18, 1895, before the chemical section of the Franklin Institute (Journal of the Franklin Institute, Vol. 140, pp. 221-237, September, 1895). While

the indefiniteness of the author's description of operations and results renders it impossible to repeat or reproduce them with any certainty, many of his conclusions are in themselves demonstrably erroneous, or rest on manifestly insufficient premises, while others are such as naturally to discourage all expectation of useful products from gilsonite.

Day's work avowedly failed of attaining the definite information that he sought regarding the nature of gilsonite; and his own tentative conclusions go very little further than that distillation of gilsonite is unpromising, and that future work on the substance should be along the lines of direct treatment with reagents such as nitric and sulphuric acids, according to a method "outlined" as a result of his investigation. While the indefiniteness of his descriptions makes any attempt to repeat or reproduce his work quite futile, such data and results as he does report, nevertheless, show very clearly that he could not really have been working with true gilsonite at all,—except, perhaps, in admixture with dominant amounts of other substances. Thus he states that the material on which he worked was lighter than water, whereas in fact gilsonite is heavier; that when heated, his material gave a final, irreducible residue of some 43%, whereas gilsonite yields no more than 30% of residue that all the volatile matter driven off by distillation was condensable by water cooling, whereas gilsonite yields such substantial proportions as some 15% of vapor not so condensable, including some 13% of well known gases; that no solid separated out in any of his redistillations, whereas, under the conditions of some of them he would have obtained from gilsonite, a hard, crystalline wax, higher melting than paraffine; that his material contained but 0.32% of both oxygen and nitrogen together, whereas gilsonite contains about 2 to 3% of nitrogen alone; and that his refining operations consumed a proportion of the oil treated that is almost unbelievable. It is also noteworthy that he does not mention the peculiar con-

2 choidal fracture so characteristic of gilsonite.

In a later paper (Am. Philosophical Society, Proc., Vol. 37, pp. 171-174; 1898), Day tells of making, by distillation of pine sawdust and fresh herring, a substance which he found practically indistinguishable from native gilsonite.

I have discovered that, by suitable treatment, giving rise to phenomena and results quite different from any thing indicated by Day, and itself also very different in many respects, gilsonite can be made the chemical basis for the production of a great variety of commercially useful products, and that it is possible to do this in such a way that almost the entire substance of gilsonite will reappear in the form of such products. As intimated above, many of my products are quite new in themselves, both chemically and physically.

All this will be fully elucidated by my description hereinafter of the best practical mode of procedure for the purposes of my invention at present known to me, and of its results, while the real scope and essence of the invention will be indicated in my claims.

The figure is a flow sheet beginning with crude gilsonite. It shows the steps of the process and their relation to each other with the products derived from the process.

While physically homogeneous and of relatively simple composition, chemically gilsonite is highly complex. Not only does chemical analysis show that it contains a number of different elements, but there are many indications that its characteristic molecule (or molecules) are of very high molecular weight and of corresponding structural complexity. According to my invention, I break up or decompose this complex material in such a way that there may be obtained and segregated or collected separately a number of different products and classes of products. Of these, part have the character of permanent gases or vapors uncondensable at ordinary temperatures; part are vapors condensable as liquid, mostly oil; and part in the form of solid coke. The gaseous portion is of such a character as to be at once serviceable as fuel or as an illuminant; but it is of considerable complexity, and can be made to yield nitrogenous and other useful products without impairment of its combustive utility. The coke is not only susceptible of direct use as fuel, or of conversion into fuel gas (of somewhat different character from that obtained as above), but has a nitrogenous content that can readily be released and segregated in useful form as an incident to conversion of the coke into fuel gas, if the antecedent operation has been appropriately conducted.

25 The liquid products present the utmost

variety and complexity, and have, moreover, a nitrogenous content very readily segregated in useful form. Though the mixture or aggregate of them resulting from the decomposition is, indeed, at once directly utilizable, their specific properties are so diverse that they can generally be utilized to the best advantage when more or less separated from one another,—or, at least, divided up into relatively homogeneous lots or fractions, so 75 to speak. These fractions may then be used directly; or further treated to bring them into a more useful state; or made the basis or raw material for the preparation of other valuable products.

In its more complete or integrated form (designed to recover or utilize the entire substance of gilsonite as fully and advantageously as may be), my process involves a first main step that is most readily carried 80 out by progressive distillation of the gilsonite destructive in character, together with further or subsidiary main steps that may be carried out by combustion of the coke from the initial distillation, and by 85 redistillation of the primary crude oil distillate (repeated a number of times in some cases) in the nature of fractionation or reduction. Preferably, of course, the vapors from all distillations will be appropriately 90 chilled or otherwise treated to segregate and recover various different useful components 95 separately. From the description of my preferred mode of procedure, however, it will 100 become apparent that various benefits and advantages of my invention can be realized even when one or more of the above-indicated steps is omitted,—and even, indeed, when the vapor from the initial distillation 105 of gilsonite is not collected or condensed.

It may be noted as a point in the economy of my complete process that burning of the fuel products obtained as described above (the two lots or kinds of fuel gas, in particular) affords all the heat necessary for 110 carrying out its two main steps of distillation, so that the process is thus thermally balanced or self sustaining. Another important point is that the unconsumed portion of the reagents required or advantageously used in the treatment of the fractionated liquid products can be utilized completely and very advantageously in the segregation of the various lots or portions of nitrogenous products above mentioned.

115 The procedure which I prefer to employ is as follows:

Gilsonite as received from the mine is charged into an iron or steel still, fired with gas or oil (or otherwise suitably heated), and connected to a suitable condenser,—such as an iron pipe condenser water-cooled. Any convenient quantity of gilsonite may be charged,—say 600 pounds to several tons. The still being closed and heat applied 120

gradually, the gilsonite will liquefy and collect in the bottom of the still, and vapor and gas evolving from it will fill the top of the still and pass over into the condenser. As the heating progresses, temperature readings should be taken from time to time on the body of vapor in the upper portion of the still, as well as on the body of liquid beneath it. (Excepting as there may be special occasion for distinguishing them, I here and hereinafter comprehend mingled gases and vapors under the single term "vapor," for the sake of brevity. Otherwise, I have applied these terms in accordance with familiar popular usage, having reference to the usual state of substances at ordinary temperatures. For convenience, I refer to various stages of operations by the corresponding vapor temperatures, unless otherwise specially noted.) The effect of the progressive heating of the gilsonite is to gradually break it up and decompose it chemically, as above mentioned,—whence, mainly, the evolution of vapor. It is a difficult matter to describe the process, or to determine in what order various products are formed or come off, since the coming off of particular products depends on the stability under heat of the highly complex chemical combinations amongst the constituents of gilsonite, as well as upon the boiling points of the products themselves. The matter is further complicated, no doubt, by the liberation, formation, and decomposition of intermediate products, both in the body of liquid and in the body of vapor. However, the coming off of vapor from the still begins at a temperature of some 165° F., and continues up to or even beyond coking temperatures. As hereinafter indicated, there is a yield of some 15% of vapor not condensable by ordinary water-cooling, including some 13% of gases. The yield of oil vapor includes a minor amount of heavy oil vapor that is condensable at relatively high temperatures, and is thick and gummy at ordinary temperatures, appropriate for condensing the bulk of the total amount of oil vapor. It is of interest to note that the distillation gas has a greater proportionate nitrogenous content than that from any hydrocarbonaceous material.

Up to the point where the vapor temperature approaches some 550° F., the distillation may be carried out as rapidly as the contents of the still can be made to absorb heat. At this point, however, some exothermic or other peculiar action occurs, so that the evolution of vapor in the still tends to become excessively rapid. Unless, therefore, the previous heating has been especially slow, it is necessary to reduce the application of heat very greatly as this critical point is approached, in order that the then undistilled liquid residue may not spew out

of the still, so to speak, and thus be carried over into the condenser, and clog it up so as to render it unusable. In practice, it will usually be found convenient to cut down the fire some 100° F. in advance of this temperature. Once this critical point is well passed, the fire may be increased and the distillation pushed on as rapidly as desired to its conclusion.

Care should be taken that the solid coke product in the still shall not reach a higher temperature than 1000° F., which is just about the temperature of initial combustion or kindling of the coke in order to avoid such fixation of the nitrogen remaining therein as would tend to defeat subsequent operations for its extraction or recovery in useful form. In practice, it will not be found necessary to exceed a temperature of some 850° F. for this material. When heated to such temperatures, this gilsonitic coke may be distinctively characterized as "dry," since it is solid and stable, and will not fuse and run.

While the vapor coming off from the still may all be led into the iron pipe condenser, as above suggested, and all of the strictly vaporous portion thereof there condensed and collected as a liquid, a slightly different procedure is preferable. As already stated, a minor portion of the vapor is condensable at relatively high temperatures; and at the temperatures in the condenser appropriate for condensing other portions, the corresponding condensate is of such thick, gummy consistency that it would tend to clog it up. It is desirable, therefore, that this heavier portion of the normally liquid products be preliminarily condensed and collected separately, without entering the condenser at all. This can advantageously be taken care of by making the pipe leading from the still to the condenser of substantial length and providing it with a trap. With this arrangement, this troublesome minor portion of the distillation products will be condensed by the cooling effect of the atmosphere upon the pipe (which thus acts as a sort of auxiliary condenser), and will collect in the trap, whence it can be drawn off from time to time and added to the liquid products drawn from the condenser itself. In other words, the distillation vapor is first chilled preliminarily in the auxiliary condenser to condense and separate out this heavier, higher boiling portion, and then further chilled in the main condenser to condense other portions. The trap also affords a measure of protection against the spewing effects of too rapid heating at the critical temperature above mentioned.

The truly gaseous portion of the distillation products will pass uncondensed through the condenser and be collected separately. The nitrogenous portion of this gas can be

segregated and secured in the form of aqueous ammonia or of ammonium sulphate, by subjecting the gas to an aqueous or a sulphuric acid scrubbing operation.

- 5 The gas thus scrubbed contains a relatively small amount of light hydrocarbon oil, unrecoverable by the ordinary water cooling described above, suspended or otherwise present therein; this may be allowed to 10 remain in order to enhance the luminosity of the gas. It may, on the other hand, be separated out and secured by a scrubbing operation with a light oil (such as spindle oil) and subsequent distillation of this oil. If 15 this oil-scrubbing is resorted to, it should preferably be done prior to the water or sulphuric acid scrubbing.

Taking representative percentages, the products into which the gilsonite is converted by the first step of my process are about 20 as follows:

|                            |       |
|----------------------------|-------|
| Light hydrocarbon oil      | 2     |
| Ammonia (NH <sub>3</sub> ) | .25   |
| Hydrocarbon fuel gas       | 12.75 |
| Distillate                 | 55    |
| Coke                       | 30    |

In the absence of the oil-scrubbing operation, the hydrocarbon fuel gas from the 30 primary distillation is a mixture with an average heating value of as high as 930 B. t. u. per cubic foot. It contains methane and other hydrocarbons, so that it can be burned with a luminous flame or used to enrich and render luminous other fuel gas. 35 Because of its hydrocarbon content, it may conveniently be distinguished as "hydrocarbon" fuel gas. Its average percentage composition is about as follows:

|                        |      |
|------------------------|------|
| CO <sub>2</sub>        | 2.8  |
| Illuminant hydrocarbon | 6.6  |
| O                      | .4   |
| CO                     | 5.8  |
| CH <sub>4</sub>        | 77.6 |
| H                      | 4.5  |
| N                      | 2.3  |

The hydrocarbon oil distillate extracted 50 from the gas by the oil-scrubbing operation is a very light, colorless, volatile liquid, vaporizing rapidly at ordinary temperature, and boiling from 80° F. to 200° F. It is suitable, in general, for the same purposes as similarly low-boiling hydrocarbons now 55 on the market,—such as conversion into illuminating gas in small isolated plants.

The nitrogen-bearing coke that collects 60 in the bottom of the still can be broken up and removed at the conclusion of the distillation, after it has cooled sufficiently. It is of interest to observe that unless this 65 nitrogenous coke has been "superheated" beyond the temperature range indicated above, its unfixed nitrogen content is quite substantial, exceeding 1%, and, in fact, amount-

ing to some 5 or 6%, which is about 80% of the total nitrogen content of the original gilsonite. This is an unprecedentedly high nitrogen content and ratio of retention for a distillation coke from a hydrocarbonaceous material. This coke may be gasified by incomplete combustion in a by-product gas-producer, its nitrogen thereby released as ammonia, unless, of course, it has been "fixed" by superheating of the coke beyond 70 such limits as above indicated. This portion of the producer gas may be separated from the remainder and recovered (by means of a water or sulphuric acid scrubbing operation) in the form of aqueous ammonia or of ammonium sulphate. Practically all of the coke is used up in the gas producer treatment,—the ash amounting to but a trifling 2 to 4%.

The significance of the above-mentioned upper temperature limit of 1000° F. for the coke during distillation and its coincidence with the initial combustion or kindling temperature of the latter may now be readily understood, by considering that in order to 80 release nitrogenous products in the gas producer, it is naturally necessary to surpass the limit of the distillation, during which the nitrogen amenable to all temperatures then attained was driven off in the distillation vapor. Such nitrogen as fails to come off at the lower temperatures attained in gas producer combustion continues its fixation under the higher temperatures there subsequently attained, and eventually comes off 90 only in forms (other than ammonia) in which is not usefully recoverable. It will also be seen that the lower the final or maximum temperature of the coke in the distillation the greater its possible nitrogen content,—which for the limit of distillation temperature above indicated will be unfixed and releasable for recovery as ammonia. In other words, the unfixed nitrogen content of such gilsonitic coke corresponds to the 100 maximum temperature to which the coke is subjected in the distillation.

It will be apparent, therefore, that my technique of controlling the distillation with reference to releasability of nitrogen from 115 the coke involves a sharp departure from ordinary practice in the treatment of hydrocarbonaceous material, according to which distillation is pushed to the utmost limit with a view to getting out as much ammonia, 120 and oil, etc., as possible in the distillation vapors, and the coke left to take care of itself.

The remainder of the producer gas, after 130 the scrubbing operation for extraction of ammonia, is a mixture of carbon monoxide, carbon dioxide, hydrogen, nitrogen, etc., suitable for use as fuel gas, and conveniently distinguishable as "carbonaceous" fuel gas. It has a fuel value of about 140 B. t. u. per

cubic foot, and is practically non-luminous. A portion of this secondary fuel gas may be satisfactorily enriched and rendered luminous by mixture therewith of the primary "hydrocarbon" fuel gas.

The average percentage composition of this secondary fuel gas from the coke is about as follows:

|    |                        |     |
|----|------------------------|-----|
| 10 | CO <sub>2</sub>        | 15  |
|    | CO                     | 11  |
|    | CH <sub>4</sub>        | 3.5 |
|    | H                      | 24  |
|    | N                      | 46  |
| 15 | Illuminant hydrocarbon | .5  |

The total liquid distillate (i. e., the mixture of the portions drawn off from the condenser and the trap) contains some 2 to 5% of water, and in this water is dissolved the 20 nitrogenous content of the crude distillate above referred to, in the form of ammonia. This water may easily be eliminated and the aqueous ammonia segregated and secured by allowing the water to settle out in a settling 25 tank. If desired, it may be converted into ammonium sulphate by means of sulphuric acid.

As it comes from the settling tank, the primary crude distillate is a reddish brown 30 oil with a green fluorescence, decidedly liquid at ordinary atmospheric temperatures, and having a specific gravity of about .875 at 60° F. After standing awhile, it loses 35 its fluorescence and becomes dark brown to black, and absolutely opaque in sections of any considerable thickness. It has a characteristic pungent odor, difficult to define, and rather unpleasant. It begins to boil at about 140° F. and distills completely below 40 700° F.; it flashes in the air at ordinary temperatures. It contains a very high percentage of unsaturated hydrocarbons,—usually about 60%, as well as combined nitrogen in proportions (some 0.2%) that are likewise unprecedentedly high as compared with other 45 mineral oils. It also contains relatively high proportions of the wax hereinafter mentioned, amounting to some 1%. It is immiscible and insoluble in water, but completely soluble in benzole and carbon-bisulphide, and miscible in all proportions with petroleum and petroleum products, turpentine, and pine oil. It presents a remarkable 50 combination of paraffinic characteristics with asphaltic ones such as hereinafter particularly pointed out with reference to lubricating oils obtainable from it. It is useful as a flotation reagent for the treatment 55 of ores by the flotation process, especially on account of its favorable ratio as between 60 saturated and unsaturated hydrocarbons.

As already intimated above, this crude oil distillate is a highly complex material, capable of fractionation to an almost unlimited extent. The different products thus

obtainable from it not only exhibit diverse properties which fit them for a great variety of industrial uses, but are susceptible of chemical treatment; purification, modification, and conversion to yield a great variety 70 of new and useful substances and materials. In practice, it is most advantageous to initially separate the crude oil into a comparatively small number of fractions, by redistillation in a suitably heated iron or steel 75 still. The redistillates may, if desired, be further purified by treatment, preferably with sulphuric acid and subsequent neutralization of the excess of reagent with alkali, such as caustic soda in aqueous solution. 80 The following examples (wherein the temperatures given are the vapor temperatures in the still, unless otherwise stated) will sufficiently illustrate the most convenient methods of redistillation:

(1) Condense separately the vapors coming from the still up to 475° F. and from 475° F. to 600° F.,—subsequently drawing off as residuum the oil unvaporized at the latter temperature, or allowing it to remain 90 and mix with the next charge of crude distillate.

(2) Condense separately the vapors up to 475° F.; from 475° F. to 650° F.; and from 650° F. until the temperature of the material in the bottom of the still is about 850° F. By this procedure, an amount of coke equal to about 2% of the crude oil charge will be produced; it may be treated in the gas-producer along with that from the primary distillation. The percentages of the products thus obtained are about as follows:

|                  |     |
|------------------|-----|
| Light oil        | 24  |
| Medium oil       | 35  |
| Heavy oil        | 36  |
| Coke             | 2.5 |
| Gas, water, etc. | 3.5 |

In either of these cases, considerable destructive action occurs in the production of 110 the higher fractions,—especially the last.

(3) Three fractions nearly similar to those described under (2) may be obtained at temperatures some 100° F. lower than those mentioned by carrying out the redistillation as described in U. S. Patent 877,620, granted Jan. 28, 1908, to Wells, blowing carbon dioxide or other inert permanent gas through the liquid in the still. In this case, the destructive action is much less. It is 115 advantageous to pass the gas and vapor coming off through a filter of fuller's earth in the dome of the still, on its way to the condenser. A residuum of heavy oil will preferably be left in the still, as described 120 under (1).

The light distillate produced in any of these ways is a yellow oil which becomes red on standing. After sulphuric acid purification, it may be desirable to redistill it re- 125

ductively in order to improve its color,— leaving as residuum in the still the small portion of the oil not coming off below 425° F. The reduced and resultant purified 5 product is a light, colorless, completely volatile oil; with mild "Terpene" odor slightly suggesting turpentine; of specific gravity about .74 to .78; and of exceptionally high and diverse solvent capacity for substances 10 used in the paint and varnish industry: specifically, its solvent capacity for varnish gums is substantially greater than that of the most similar petroleum derivatives. Its terpene characteristic is considerably more 15 marked than in the case of refined petroleum, especially after prolonged standing. The intermediate distillate oil is a yellow oil with green fluorescence when fresh; on standing, it becomes first red and then, even- 20 tually, a deep reddish brown. Its specific gravity is about .870. It is capable of use as gas oil or fuel oil without sulphuric acid purification. It is more reactive to sul- 25 phonating reagents than the most similar mineral oil distillates from petroleum or other known hydrocarbonaceous material. It is susceptible of sulphonation treatment with oil of vitriol and oleum (preferably after preliminary purification with a small 30 percentage of oil of vitriol) to yield various useful products. These include a residual which after neutralization and redistillation is a thin, clear oil, substantially colorless, odorless, and tasteless; a sulphonation 35 reaction oil of highly useful semi-drying properties; and a water-soluble product with the useful properties (hydrolyzing, detergent, emulsifying) generally characteristic of true sulphonic substances. These last two 40 products can be segregated by diluting the sulphonation sludge with an equal amount of water and allowing the solution to stand at a temperature of 150° F. and separate into layers by gravity. Of the resultant 45 layers, the top comprises the reaction oil and the middle the aforesaid water-soluble sulphonated product, while the bottom comprises most of the unconsumed sulphuric acid diluted with water. The middle layer 50 may be freed from contaminating organic impurity by neutralization, which sets the impurity free to rise to the surface and be removed,—or, in like manner, by free dilution with water.

55 The heavy distillate oil is a somewhat viscous reddish-yellow oil with green fluorescence when freshly prepared; on standing, it becomes almost black,—or brown in a thin film. Its specific gravity is about .927.

60 Both it and the residual oil redistillate (if produced) are suitable for use as flotation reagent without further treatment. The residual oil has a specific gravity of about .933.

65 These gilsonite oil fractions or redistillates have the same strikingly high content

of combined nitrogen and of unsaturated hydrocarbons as the crude primary distillate described above, and the higher boiling fractions contain the gilsonitic wax referred to. The peculiar combination of paraffinic and asphaltic properties is even more marked in the high boiling fractions than in the crude distillate itself.

The heavy distillate is suitable for the manufacture of lubricating oil. For this purpose, it may be purified by treatment with 3 to 10% of oil of vitriol; neutralized with caustic soda or other alkali; washed with water; and then chilled to about 32° F. and filter-pressed. This pressing removes 80 from the oil a material which, after repressing and filtering through fuller's earth, becomes a merchantable wax, hard and crystalline, dark yellow to reddish in color, with a melting point of about 135° F. to 170° F. as compared with 120° F. for paraffine. The pressed oil is then fractionated or reduced according to the particular variety of lubricant desired. The resultant products are viscous, yellowish red oils, with pronounced 90 green fluorescence; they have specific gravities of 0.9 and upward; they give a flash test of not less than about 350° F.; they boil at temperatures exceeding 45° F., and, for the most part, above 600° F. They are stable against decomposition into products 95 unsuited to lubrication under even the unfavorable conditions of internal combustion engine cylinder lubrication; and they are inert with respect to ordinary metals, so that they will not injure machine parts. Contrary to the "paraffinic" character indicated by the wax obtained from their "mother oil", so to speak, they have, it will be observed, the relation of flash point to specific 100 gravity generally characteristic of asphaltic oils. This will readily be observed by comparing their properties as stated with those 105 of commercial petroleum lubricating oils:

|         | California<br>asphaltic. | Paraffinic. | Gilsonitic. |
|---------|--------------------------|-------------|-------------|
| Density | .91                      | .87         | .9          |
| Flash   | 395                      | 400         | 350         |

Thus it will be observed that for similar 115 gravities the asphaltic and gilsonitic lubricating oils have flash points below those for even lighter paraffinic oils.

The unconsumed portion of the sulphuric acid or other such reagent used in the various purifying and sulphonation treatments above described can be used as a reagent for the segregation of nitrogenous products from the primary gas, liquid, and coke products as above set forth. Sulphonation of the intermediate distillate described above will afford enough such unconsumed acid for this purpose.

Having thus described my invention, I 130 claim:

1. A process of converting gilsonite into oils, ammonia and fuel gas, which comprises heating and thereby decomposing and distilling the gilsonite to dryness, at increasing temperatures below that of nitrogen fixation in the resulting coke, to yield dry coke retaining nitrogen of the gilsonite unfixed and also vapor comprising segregable fuel gas, ammonia, and oil vapor, the latter including portions one of which is condensable at higher temperatures than the other and is thick and gummy at temperatures at which such other condenses; reducing the application of heat for distillation as the vapor temperature over the then undistilled residue approaches and passes 550° F.; and withdrawing vapor as formed from the presence of the undistilled residue, and chilling such vapor preliminarily to condense and separate out the thick, gummy portion aforesaid, and further to condense the other portion.

2. A process of converting gilsonite into oils, ammonia, and other gas, which comprises heating and thereby decomposing and distilling the gilsonite to dryness, at increasing temperatures below that of nitrogen fixation in the resulting coke, to yield dry coke with nitrogen content releasable as ammonia and also vapor comprising free ammonia, other gas in substantial proportions, and oil vapor; and burning the aforesaid coke and releasing its nitrogen content as ammonia.

3. A process which comprises heating and thereby decomposing and distilling gilsonite to coke, at increasing temperatures below that of nitrogen fixation in the coke, to yield coke retaining nitrogen of the gilsonite unfixed and also oil vapor, portions of which are condensable at higher temperatures than other portions and are thick and gummy at temperatures at which said latter portions condense; withdrawing the vapor as formed from the presence of the undistilled residue, and preliminarily condensing and separating out the thick, gummy portions aforesaid, and then condensing the other portions.

4. A process which comprises heating and coking gilsonite within such limits of maximum temperature as to retain nitrogen of the gilsonite in the coke unfixed, and treating the coke to release such retained nitrogen as ammonia.

5. A process which comprises heating and thereby decomposing and distilling gilsonite to solid coke, at increasing temperatures below that of nitrogen fixation in the coke, and releasing such retained nitrogen as ammonia through incomplete combustion of the coke at temperatures exceeding the previous limit.

6. A process of obtaining nitrogenous products from gilsonite which comprises heating and thereby decomposing and cok-

ing the gilsonite, with incidental nitrogenous yield, within such limits of maximum temperature of the coke as to retain therein a maximum proportion of nitrogen, and treating the coke to release such retained nitrogen as ammonia.

7. A process which comprises heating and thereby decomposing and distilling gilsonite, to yield gas in substantial proportions and oil distillate, and fractionally redistilling such distillate to yield more homogeneous fractions, the high fractions containing hard, crystalline wax and stable, inert, viscous lubricating oils of paraffinic character, having asphaltic relations of flash point to specific gravity.

8. A process which comprises heating and thereby decomposing and distilling gilsonite at increasing temperatures eventually exceeding 550° F. for the vapor over the undistilled residue, to yield oil vapor including portions one of which is condensable at higher temperatures than the other and is thick and gummy at temperatures at which such other condenses, reducing the application of heat as the vapor temperature over the residue approaches and passes 550° F.; and progressively withdrawing the vapor from the presence of the undistilled residue, and preliminarily condensing and separating out the thick, gummy portion aforesaid, and then condensing the other portion.

9. A process which comprises heating and thereby decomposing and distilling gilsonite to yield oil vapor including portions one of which is condensable at higher temperatures than the other and is thick and gummy at temperatures at which such other condenses; and withdrawing the vapor from the presence of the undistilled residue, and preliminarily condensing and separating out the thick, gummy portion aforesaid, and then condensing the other portion.

10. A process which comprises heating and thereby decomposing and distilling gilsonite at increasing temperatures eventually exceeding materially 550° F. for the vapor over the undistilled residue, materially reducing the application of heat, however, as such vapor temperature approaches and passes that figure.

11. A process which comprises heating and thereby decomposing and distilling gilsonite until the undistilled residue is coked, at increasing temperatures below that of nitrogen fixation in the coke, to yield coke with nitrogen content releasable as ammonia and also vapor comprising segregable oil vapor and gas; reducing the application of heat, however, as the vapor temperature over the then undistilled residue approaches and passes 550° F.

12. A process of producing, from gilsonite, coke with nitrogen content recoverable as ammonia, and other useful products,

which comprises heating and thereby destructively distilling the gilsonite to solid, non-melting coke, at increasing temperatures below that of nitrogen fixation in the coke.

13. A process of obtaining, from gilsonite, non-melting coke with recoverable nitrogen content, which comprises heating and thereby decomposing and coking the gilsonite at increasing temperatures up to a maximum of from 850° F. to 1000° F.

14. A process which comprises heating and thereby decomposing and coking gilsonite at increasing temperatures, with a maximum, for the residue, of some 850° F., to yield dry, solid coke with corresponding unfixed nitrogen content.

15. A process which comprises heating and thereby decomposing and distilling gilsonite, at increasing temperatures eventually exceeding 550° F. for the vapor over the then undistilled residue, until the residue is coked.

16. A process which comprises heating and thereby decomposing and distilling gilsonite until the undistilled residue is coked,

at increasing temperatures eventually exceeding 550° F., but below that of nitrogen fixation in the coke.

17. A process which comprises heating and thereby decomposing and distilling gilsonite at increasing temperatures yielding oil vapors of varying boiling points up to and including a high-boiling portion that is thick and gummy at temperatures at 35 which the low-boiling portion condenses, and also gas in substantial proportions.

18. A process which comprises heating and thereby decomposing and distilling gilsonite at increasing temperatures eventually sufficiently high to yield distillate comprising hard, crystalline wax of very high melting point and also stable, inert, viscous lubricating oils of paraffinic character and asphaltic relations of flash to specific gravity, 40 and for the most part boiling below 600° F., besides gas in substantial proportions.

In testimony whereof, I have hereunto signed my name at Philadelphia, Pennsylvania, this twelfth day of August, 1919.

CHARLES N. FORREST.